

## UNITED STATES PATENT OFFICE

2,629,676

## CORROSION INHIBITORS

Carl F. Prutton, New York, N. Y., assignor to The Lubrizol Corporation, Wickliffe, Ohio, a corporation of Ohio

No Drawing. Application September 2, 1949,  
Serial No. 113,909

9 Claims. (Cl. 148—6.17)

1

This application is a continuation-in-part of my copending application, Serial No. 671,123, filed May 20, 1946, now abandoned, which in turn was a continuation-in-part of my then copending application, Serial No. 369,227, filed December 9, 1940, now Patent No. 2,400,573, dated May 21, 1946; which application was a continuation-in-part of my then copending application Serial No. 99,165, filed September 2, 1936, now abandoned.

The present invention relates to the art of treating metal and is particularly directed to an improved method of the treatment of metal surfaces to prevent corrosion and rust.

Many attempts are known in the prior art to provide rust and corrosion inhibitors for metals, but these efforts heretofore have either proved unsatisfactory or too expensive in practice to warrant their wide commercial adoption.

In general, objects of this invention are to provide a coating composition which is very stable in its use and application; one that is usable for metals directly without preliminary treatment or finishing operations; a compound which is inexpensive and generally reduces the cost of coating metal.

The specific object hereof is to provide a compound which will react with the metal to which it is applied to efficiently protect the surface of such metal and effectively prevent oxidation and corrosion.

In accordance with the present invention, I have discovered that certain phosphorus-containing compounds, generally known as the phosphide compounds, in non-aqueous media are readily applicable to metal surfaces to inhibit corrosion action. More particularly, this invention is concerned with organic phosphide types of compounds containing a metal group, and still more specifically the organo-metallic phosphides. For most purposes, it is preferred to employ an organo-metallic phosphide of such nature that in contact with an aqueous media they will yield a solution having a pH of below about 7, my research and tests showing the most satisfactory results to be when the pH is between about 4 and 6, in most cases. For reasons not too clearly understood the organo-metallic phosphides give particularly good results in inhibiting corrosion of such metals as for example ferrous types, bearing metals of copper-lead, cadmium-silver, or analogous types.

For the purposes of this specification and the appended claims, the term "organometallic phosphide" is intended to include those compounds in which the metal substituent is solely attached to

2

the phosphorus atom, and such compounds must contain at least one organic radical attached to the phosphorus atom.

Generally, the organo-metallic phosphides can be represented by the following structural formula:

(a)  $M_aPbR_c$

10 where M is a mono-, di- or polyvalent metal, R is an organic radicle, hydrogen, or halogen, at least one of which is an organic radicle, and "a" and "b" can be either one or two, and "c" can be up to 4, depending on the valence of the metal. To illustrate this point, when M is a divalent metal, "a" is 1, "b" can be either 1 or 2, and "c" can be either 1 or 4, in accordance with the following subgeneric structural formulae:

20 (b)  $M=P-R$

(c)  $M=\left( \begin{array}{c} R \\ | \\ P \\ | \\ R \end{array} \right)$

25 In the case of a monovalent metal represented by M in the above structural Formula (a), the numerical values of "a" and "b" and "c" in said formula will vary in accordance with the following subgeneric structural formulae:

30 (d)  $\begin{array}{c} M \\ | \\ P-R \\ | \\ M \end{array}$

35 (e)  $M-P=R_2$

The organo-metallic phosphides can have present therein metals from groups I and II of the periodic system, namely the alkali or alkaline 40 earth metals. Other polyvalent metals also can be suitably employed, however, it is preferable to use metals from groups I and II of the periodic system.

The halogen present in the phosphides of this 45 invention generally can be of any halogen, but it is preferred to employ chlorine as the halogen contained in the organo-metallic phosphides.

The organic radicles as previously mentioned 50 can be one or more "R's" in the generic structural Formula (a) given hereinabove. In a more particular identification of the types of organic radicles present in the organo-metallic phosphides, the table below enumerates examples thereof in an order of convenience rather than preference. It is preferred to employ oil solu-

bilizing organic radicles, which contain a plural-  
ity of carbon atoms, advantageously about 4  
or more.

TABLE I  
*Organic radicles*

|                              |                                                                                                                           |
|------------------------------|---------------------------------------------------------------------------------------------------------------------------|
| I. Aliphatic                 | A. Hydrocarbon                                                                                                            |
|                              | 1. Acyclic                                                                                                                |
|                              | a. propyl                                                                                                                 |
|                              | b. butyl                                                                                                                  |
|                              | c. amyl                                                                                                                   |
|                              | d. the radicles of other homologous com-<br>pounds enumerated above.                                                      |
|                              | 2. Cyclic                                                                                                                 |
|                              | a. Cycloparaffins                                                                                                         |
|                              | (1) cyclopentyl                                                                                                           |
|                              | (2) cyclohexyl                                                                                                            |
| II. Aromatic                 | A. Benzene series                                                                                                         |
|                              | (1) phenyl                                                                                                                |
|                              | (2) methyl phenyl                                                                                                         |
|                              | (3) radicles of other homologous compounds<br>of benzene                                                                  |
|                              | B. Naphthalene series                                                                                                     |
|                              | (1) naphthyl                                                                                                              |
|                              | (2) methyl naphthyl                                                                                                       |
|                              | (3) other homologous radicles of naphthalene                                                                              |
| III. Oxygen bearing radicles | The OR group where R can be any of the aliphatic<br>radicles enumerated under I and II                                    |
| IV. Halogen bearing radicles | The halogen, for example chlorine, can be present<br>in any of the organic radicles listed under I, II,<br>and III above. |

Examples of organo-metallic phosphides found  
applicable for the purposes of this invention in-  
clude:

Calcium amyl phosphide  
Barium octyl phosphide  
Zinc octyl phosphide  
Barium cresyl phosphide  
Barium benzyl phosphide  
Magnesium chlorophenyl phosphide  
Phenyl lead phosphide

It is not to be inferred that all organo-metallic  
phosphides are equivalent in efficacy, but that  
under certain conditions some organo-metallic  
phosphides are more desirable than others.

In order that a better understanding can be  
obtained of my invention, two illustrative ex-  
amples of methods of preparation will be given.  
It should be understood that the examples are  
given by way of illustration and not by way of  
limitation.

An organic phosphine which may be either  
 $RPH_2$  or  $R_2PH$  is reacted with an alkali metal  
such as sodium or potassium to produce a phos-  
phide. The alkali metal is dissolved in liquid  
ammonia. The alkali dissolves in liquid am-  
monia without reaction. The organic phosphine  
is then introduced slowly into the solution.  
When using an organic phosphine of the  
formula  $RPH_2$  and when using equal molecular  
portions of the organic phosphine and metal  
there will be produced a compound having the  
formula  $RPHM$ . However, when 1 mol of the  
organic phosphine  $RPH_2$  is combined with 2 mols  
of the metal, a phosphide having the formula  
 $RPM_2$  is produced. When utilizing an organic  
phosphine of the formula  $R_2PH$ , 1 mol thereof  
will be used for a mol of metal and the phosphide  
produced will have the formula  $R_2FM$ .

A second method for the preparation of the  
phosphides is by means of the reaction of an  
organic phosphine with zinc diethyl. Accord-  
ingly, to this method an organic phosphine of  
the formula  $RPH_2$  is introduced to the liquid  
zinc diethyl and at room temperature or only

slightly above room temperature the reaction  
will proceed to the production of



10 When using an organic phosphine of the for-  
mula  $R_2PH$  the reaction thereof with zinc di-  
ethyl will result in the following:



15 A further advantage of the present discovery  
in the compatibility of certain organo-metallic  
phosphides in relatively pure state with oils and  
with vehicles used in coating materials, such as  
paints, varnishes, lacquers; and with other sol-  
vents partly or wholly immiscible with water.  
20 This is especially valuable in carrying out the  
invention as the corrosion inhibiting compound  
may be included in ornamental or preservative  
coating mixtures and applied to the surface to  
be treated without an extra operation. Still fur-  
ther, it has been found that the affinity of organo-  
metallic phosphide compounds with paint, var-  
nish, and lacquer coating materials generally  
improves the resulting coating and provides an  
effective bond or adherence thereof to the surface  
of the metal due to the reaction of such com-  
pounds with the metal.

25 In practice, a metal surface may be treated  
with an organo-metallic phosphide in an oil or  
30 other carrying vehicle to provide a thin coating  
on such surface. One very effective method  
comprises heating a coating liquid to a suitable  
temperature, immersing the article to be pro-  
tected, and then cooling or drying in air the thin  
35 adherent coating upon the article which resulted  
from the bath. The drying may be accelerated  
by placing the coated article in a suitable oven.

40 The novel coating compound is preferably car-  
ried in non-aqueous media, such as petroleum  
45 oils and solvents, fatty oils, greases, waxes, or  
other organic solvents, or mixtures of the above  
such as are used as vehicles for paints, var-  
nishes, lacquers, etc. Such compound will then  
50 react by itself or in contact with water or with  
the surface of the metal to which the coating  
is applied, to produce thereon a protective coat-  
ing. It has been found that certain of these  
55 organo-metallic phosphides will attack the metal  
and produce a roughening of the metal and there-  
by greatly increase the adherent properties of  
such metal when an ornamental coating is ap-  
plied thereto.

60 The invention also contemplates physically  
combining with the organo-metallic phosphide  
an organic derivative of an inorganic acid, e. g.  
sulphuric acid, silicic acid, nitric acid, or the  
like. These hydrolyzing agents are found to  
65 accelerate the attack on the metal surface and  
to greatly enhance the properties of such surface  
to hold coatings thereon.

Examples of the above mentioned organic de-  
rivatives of inorganic acids are the silicates, nit-  
rates, sulphates, and the sulphonates and ester  
and salts of the sulphonates. The sulphonates  
and ester and salts thereof are the preferred  
derivatives of inorganic acid which may be used  
in combination with the organo-metallic phos-  
phides.

70 In the following table are listed specific ex-  
amples of types of sulphonic acids, esters and

salts which are useful in accordance with the principles of this invention.

TABLE II

## Sulphonic acids, e. g.:

Benzene sulphonic acid  
Naphthalene sulphonic acid  
Amyl naphthalene sulphonic acid  
Capryl benzene sulphonic acid  
Lauryl benzene sulphonic acid  
Lauryl sulphonic acid  
Cetyl sulphonic acid  
Petroleum mahogany sulphonic acids

## Esters of sulphonic acids, e. g.:

Butyl ester of benzene sulphonic acid  
Benzyl ester of benzene sulphonic acid  
Chlor-benzyl ester of benzene sulphonic acid  
Phenyl ester of lauryl sulphonic acid  
Ethyl ester of cetyl sulphonic acid  
Phenyl ester of petroleum mahogany sul-  
phonic acid

## Salts of sulphonic acids, e. g.:

Calcium salt of petroleum mahogany sul-  
phonic acid  
Barium salt of petroleum mahogany sul-  
phonic acid  
Magnesium salt of petroleum mahogany sul-  
phonic acid  
Aniline salt of petroleum mahogany sul-  
phonic acid  
Calcium salt of lauryl benzene sulphonic  
acid  
Zinc salt of capryl benzene sulphonic acid

From the foregoing it will be observed that the particular derivatives of sulphuric acid listed are characterized by the formula



Where M is hydrogen (acids), an organic radical (esters) or a metal (salts).

Other specific examples of the above mentioned organic derivatives of inorganic acids are:

Ethyl silicates  
Ethyl sulphuric acid  
Lauryl sulphuric acid  
Aniline sulphate

An example of the combination of one of the above with an acid compound of phosphorus is:

Sulphonated diphenyl phosphoric acid.

It is very important to note that the processes involving the admixture of the novel inhibiting compound with another coating composition provides a more satisfactory bond or means of attachment of such other composition to metal surfaces. Obviously, if an ingredient of a coating composition does in itself react with and adhere to a metal surface, then such composition carrying this ingredient will become permanently adhered to the metal when applied.

As an example of a composition which may be employed for the purposes of the present invention, calcium amyl phosphide may be employed in combination with the calcium salt of petroleum mahogany sulphonic acid in a non-aqueous oil vehicle.

As stated in the general outline of this invention, it is sometimes desirable that organo-metallic phosphides to be used as the present novel inhibitor be of such nature that in contact with water they will yield a solution having a pH of below 7, preferably below 6 and above 4. Such materials are of sufficiently acidic nature as to

react chemically with metal surfaces to form adherent protective coatings.

Because of the very nature of the organo-metallic phosphides it has been found that such agents as moisture, which ordinarily promotes corrosion, will, when attacking the metal surface treated by the present novel coating method, produce an accelerated reaction of such organo-metallic phosphides used in the coating with the metal to form a thin protective layer.

While I have presented theories to explain the action of organo-metallic phosphides as corrosion inhibitors, it should be understood that I do not intend to be bound thereby. The theories have been solely presented with the view of aiding the advancement of the arts as much as possible.

From the above description, it has been shown that the compounds described, when incorporated in a coating composition, are all effective and desirable corrosion and oxidation inhibitors.

The present invention is not limited to the specific embodiments of the present invention and not limitations of the scope thereof. Likewise the quantities of materials employed and the procedure of preparation may be widely varied without departing from the scope of this invention, nor is it intended to limit the use of any member of the new class of inhibitors to any particular coating composition. The present invention is limited solely by the claims attached as a part of this specification.

The amount of the above-described organo-metallic phosphides required for my purpose depends upon the nature of the compound, the kind of use, and the character of the vehicle. In the case of certain of the more active compounds, a very low percentage is sufficient, e. g. from 0.01 to 0.25%, and for most purposes, amounts up to about 5% are desirable. Usually only a minor amount need be used; but in the case of certain of the materials, for example, particularly those useful as pigments or fillers much higher proportions, up to 90% or more, may be found useful.

Other modes of applying the principle of the invention may be employed, change being made as regards the details described, provided the features stated in any of the following claims or the equivalent of such be employed.

I therefore particularly point out and distinctly claim as my invention:

1. A corrosion inhibitor for metal surfaces comprising the combination of an oil-soluble organo-metallic phosphide, which compound has a metal substituent solely attached to phosphorus and contains at least one organic radical selected from the class consisting of hydrocarbon and halogen-containing hydrocarbon radicals, and a non-aqueous oil vehicle.

2. The corrosion inhibitor of claim 1 is further characterized by yielding a pH value below 7 when in contact with an aqueous media.

3. A corrosion inhibitor for metal surfaces comprising the combination of an oil-soluble organo-metallic phosphide compound having the general formula  $M_aP_bR_c$  wherein M is a metal solely attached to P and R is selected from the group consisting of hydrogen, halogen, hydrocarbon, and halogen-containing hydrocarbon radicals having a valence of one, which compound contains at least one organic radical; a and b can be either one or two, and c is not less than one or more than four, such compound when in contact with an aqueous media yields a solu-

tion having a pH of below 7; and a non-aqueous oil vehicle.

4. A corrosion inhibitor in accordance with claim 3 in which M is a bi-valent metal.

5. A corrosion inhibitor in accordance with claim 3 in which M is a metal of group 2 of the periodic table.

6. A corrosion inhibitor for metal surfaces comprising in combination, an oil-soluble organo-metallic phosphide having the following 10 general formula:



wherein M is a bivalent metal and R is a hydrocarbon group having valence of one, which compound upon contact with an aqueous media yields a solution having a pH of below 7; and a non-aqueous oil vehicle.

7. A corrosion inhibitor for metal surfaces comprising in combination (a) an oil-soluble organo-metallic phosphide, which compound has a metal substituent solely attached to phosphorous and contains at least one organic radical selected from the class consisting of hydrocarbon and halogen-containing hydrocarbon radicals, and upon contact with an aqueous media yields a solution having a pH of below 7; (b) an organic compound selected from the group consisting of organic sulphonic acids, esters of organic sul-

phonic acids, and salts of organic sulphonic acids; and (c) a non-aqueous oil vehicle.

8. A corrosion inhibitor for metal surfaces comprising in combination (a) calcium amyl phosphide, and (b) a non-aqueous oil vehicle.

9. A corrosion inhibitor for metal surfaces comprising in combination (a) calcium amyl phosphide, (b) calcium salt of petroleum mahogany sulphonic acid, and (c) a non-aqueous oil vehicle.

CARL F. PRUTTON.

#### REFERENCES CITED

The following references are of record in the 15 file of this patent:

#### UNITED STATES PATENTS

| Number    | Name             | Date          |
|-----------|------------------|---------------|
| 2,149,271 | Butz             | Mar. 7, 1939  |
| 2,199,944 | Van Peski et al. | May 7, 1940   |
| 2,224,695 | Prutton          | Dec. 10, 1940 |
| 2,321,307 | Mikeska et al.   | June 8, 1943  |
| 2,340,331 | Knutson et al.   | Feb. 1, 1944  |
| 2,400,573 | Prutton          | May 21, 1946  |
| 2,486,664 | Marling et al.   | Nov. 1, 1949  |

#### FOREIGN PATENTS

| Number  | Country       | Date          |
|---------|---------------|---------------|
| 483,400 | Great Britain | Apr. 20, 1938 |